

## UNITED STATES PATENT OFFICE

2,036,119

## PRIMER COMPOSITION

Gordon H. Chambers, Philadelphia, Pa., assignor  
to Foote Mineral Company, Philadelphia, Pa.,  
a corporation of Pennsylvania

No Drawing. Application September 23, 1931,  
Serial No. 564,725

13 Claims. (Cl. 52—3)

My invention relates to primer compositions and the like, and is particularly adaptable and advantageous for ammunition primers and detonator caps. I have discovered that such compositions can be greatly improved by the use of zirconium in them. Besides its general advantage as a combustible and igniter in such priming mixtures, it is especially advantageous in non-corrosive ammunition primers for small-arms.

5 Zirconium in the form of fine powder ignites readily at comparatively low temperatures, thus giving easier ignitability and sensitiveness to the mixture. As it has an extremely high heat of combustion (1956.7 calories per gram), and

10 flashes very quickly (less than 1/1000 second), its flame temperature is very high. These properties of low ignition temperature and high flame temperature make zirconium very efficient for initiating the combustion or explosion of less

15 sensitive materials.

As is well understood in the explosive art, an ammunition primer or igniter is a portion of a cartridge or other explosive device (or, more properly speaking, a portion or charge of explosive) in which ignition is (percuttively or frictionally) initiated, and by which a larger explosive charge is fired thermally. In a detonator cap, likewise, the igniter—sometimes also designated a "primer"—is a part (or a charge) in

20 which ignition is thermally or electrothermally initiated, and by which an explosion is started that ultimately fires another charge by detonation. From these facts and the peculiar properties of zirconium just explained, its advantages in

25 igniter charges or primers for both types of devices—those percussively fired, and those thermally fired—may be in part appreciated.

As an example of the use of zirconium in primers, I may instance its addition to an ordinary standard composition of mercury fulminate, barium nitrate, and antimony sulphide, preferably in such substantial proportions as 10 parts, say, of commercial zirconium powder to 100 parts of the total of the aforementioned ordinary primer ingredients, by weight. In such a primer composition for ammunition, the mercury fulminate serves as a highly sensitive percussive combustion-initiator; the barium nitrate as an oxidizer, non-corrosive toward a gun barrel; and the antimony sulphide as a combustible or fuel,—though less sensitive than zirconium. Wide variation of proportions is permissible, however: e. g., an addition of as little as 2% zirconium powder will give greater ignitability to some primer mixtures; and it may, on the other hand, be used in much

larger proportions than 10%, such as 25% or more.

A further advantage of zirconium in primers or blasting caps is its great resistance or stability against deterioration. While most primer or percussion compositions tend to deteriorate under warm and damp atmospheric conditions, moderate temperatures or rises in temperature do not affect zirconium, and careful tests show that it does not deteriorate in contact with moisture. 10 Zirconium also resists the attack of many of the oxidizers and alkali compounds that are used in primer and percussion mixtures. For all of these reasons, it increases the life, efficiency, and reliability of priming and detonating compositions in 15 which it is used.

In the use of priming mixtures containing it, zirconium forms a heavy ash with some of the usual ingredients, such as barium nitrate, and thus reduces or eliminates the smoke from the 20 primer. It also appears to form a protective coating (probably a thin layer of zirconium oxide) in gun barrels,—a property which may give it special value in a non-corrosive, non-mercuric primer.

It is to be observed that commercial zirconium 25 metal powder as at present produced appears to contain a substantial proportion of impurity—probably a suboxide or hydride of zirconium—whose exact character and effect on the properties of the powder have never been definitely determined. 30 It is possible, of course, that various advantages of zirconium for my purposes (as hereinbefore set forth) are either diminished or enhanced by such "suboxide" or other impurity or dependent on its presence. Accordingly, the 35 addition or substitution of such "suboxide" to or for zirconium powder is within the scope of my invention in its broader aspects, as well as the use of zirconium without the presence of the suboxide.

Having thus described my invention, I claim:

1. A percussively fired igniter charge for an explosive charge, comprising zirconium.
2. A percussively exploded composition comprising zirconium.
3. An ammunition priming mixture containing zirconium, an oxidizer, and a combustion initiator.
4. An ammunition priming mixture containing zirconium, a non-corrosive oxidizer, and a suitable combustion initiator.
5. An ammunition priming mixture containing zirconium, a second fuel ingredient, a non-corrosive oxidizing ingredient, and a combustion initiator.

6. An ammunition priming mixture containing zirconium, and barium nitrate.
7. An ammunition priming mixture containing zirconium, barium nitrate, and mercury fulminate.
5. 8. An ammunition priming mixture containing zirconium, antimony sulphide, a suitable oxidizer, and a suitable combustion initiator.
9. An ammunition priming mixture containing zirconium as fuel.
10. 10. An ammunition priming mixture containing metallic zirconium and a non-corrosive oxidizer.
11. A non-corrosive priming mixture comprising a nitrate adapted to serve as an oxidizing agent without corrosive tendencies toward a gun barrel, and zirconium as a fuel.
12. An ammunition priming mixture containing a combustion initiator, an oxidizer, a fuel, and a small quantity of zirconium.
13. A non-corrosive priming mixture comprising a combustion initiator, a nitrate adapted to serve as an oxidizing agent without corrosive tendencies toward a gun barrel, and metallic zirconium as a fuel.

GORDON H. CHAMBERS.